

## UNITED STATES PATENT OFFICE

2,389,181

## ELECTRODEPOSITION OF METALS

Henry Brown, Kansas City, Mo., assignor to The  
Udylite Corporation, Detroit, Mich., a corpora-  
tion of Delaware

No Drawing. Application May 15, 1941,  
Serial No. 393,662

16 Claims. (Cl. 204—45)

My invention relates to improvements in the electrodeposition of metals. It is particularly concerned with the utilization of certain addition agents, for the purposes hereinafter stated, in aqueous acidic electroplating baths.

I have discovered that certain substances, hereinafter described in detail, when added to electroplating baths, particularly aqueous acidic electroplating baths such as used for the electrodeposition of nickel, cobalt, iron, zinc, cadmium, copper, antimony, various alloys containing the aforementioned and other metals, and the like, are remarkably effective in the prevention of the formation of pits in the electro-deposited coatings, said pits normally being caused by the adherence of gas bubbles during the electrodeposition of the coating. I have found, further, that this result is accomplished despite the fact that very low concentrations of the addition substances are employed and, still further, that these results are accomplished without causing any significantly appreciable interference with the desired appearance, structure, and character of the plate.

I have also discovered that the addition agents are highly effective independently of whether various organic or inorganic so-called brightening agents are also present in the electrolyte bath. Various addition agents have heretofore been suggested for reducing or eliminating pitting in electrodeposition operations but, at least in most cases, and apart from other deficiencies which they possess, they have proven to be wholly unsatisfactory where the electrodeposition bath contained brighteners. Thus, for example, in baths employed for the electrodeposition of bright nickel, where the brightening agent comprises an aryl sulphonic acid, for example, naphthalene 1,5 disulphonic acid, sodium salt, or sulphonamides or sulphonimides such as are disclosed in my Patent No. 2,191,813, issued February 27, 1940, various suggested anti-pitting agents have proven entirely unsatisfactory. The use of the addition agents in bright plating baths represents but one aspect of my present invention although, to be sure, a highly important one.

The addition agents which I have found to be unusually satisfactory, in accordance with my present invention, can be used in sufficiently low concentrations so as to reduce substantially, or eliminate entirely, pitting of the deposits and, at the same time, they do not interfere to any significantly appreciable extent with the particular cathodic process involved such as reduction of inorganic or organic substances taking place in the process of electrodepositing the coating. This is highly important where the deposited

metal is desired not only free from pits but also of maximum ductility and purity and freedom from such inclusions as sulphur, carbon and colloids. It is also of considerable importance in those cases involving bright plating baths, particularly aqueous acid plating baths for the electrodeplating of nickel, which baths contain brighteners such as those mentioned hereinabove, particularly those wherein the brightener is in the form of a soluble compound containing the radical  $-\text{SO}_2\text{N}-$ . As I have pointed out hereinabove, the brightness or brilliance or high luster of the deposits is not adversely affected where the addition agents, to which my present invention relates, are employed.

The novel and highly useful addition agents which accomplish the functions set out hereinabove are, in general, aliphatic alkyl ether sulfonates containing at least 8 carbon atoms, preferably containing an alkyl chain of 8 to 18 carbon atoms especially 12 to 14 carbon atoms.

Illustrative examples of addition agents which may be utilized in accordance with my invention are set out hereinbelow. They may be utilized in the form of the free sulfonic acid derivative but are preferably employed in the form of the sodium, potassium or ammonium salts or as the salts of the metal being deposited from the bath. In general, they are used in concentrations of the order of about 0.05 to about 0.5 gram per liter of electrolyte solution, from about 0.1 to about 0.3 gram per liter of electrolyte solution being most satisfactory in the usual case. More addition agent may be utilized but it is, in general, uneconomic to do so and fully satisfactory results are obtained in practically all cases with the preferred range set out hereinabove.

- 40 (1)  $\text{CH}_3-(\text{CH}_2)_{10}-\text{CH}_2-\text{O}-\text{CH}_2-\text{SO}_3\text{Na}$   
1-oxydodecyl-1-sodium sulfonate-methane
- (2)  $\text{CH}_3-(\text{CH}_2)_6-\text{CH}_2-\text{O}-\text{CH}_2-\text{SO}_3\text{Na}$   
1-oxyoctyl-1-sodium sulfonate methane
- (3)  $\text{CH}_3-(\text{CH}_2)_{10}-\text{CH}_2-\text{O}-\text{CH}_2-\text{CH}_2-\text{SO}_3\text{K}$   
1-oxydodecyl-2-potassium sulfonate ethane
- (4)  $\text{CH}_3-(\text{CH}_2)_{10}-\text{CH}_2-\text{O}-(\text{CH}_2)_3-\text{CH}_2-\text{SO}_3\text{NH}_4$   
1-oxydodecyl-3-ammonium sulfonate propane
- 45 (5)  $\text{CH}_3-(\text{CH}_2)_{10}-\text{CH}_2-\text{O}-\text{CH}_2-\text{CH}(\text{CH}_3)-\text{CH}_2-\text{SO}_3\text{Na}$   
1-oxyoctyl-2-hydroxy-3-sodium sulfonate propane
- (6)  $\text{CH}_3-(\text{CH}_2)_{10}-\text{CH}_2-\text{O}-\text{C}_2\text{H}_4-\text{O}-\text{C}_2\text{H}_4-\text{SO}_3\text{Na}$   
1-(dodecloxyethyl) oxy-2-sodium sulfonate ethane

- (7)  $\text{CH}_3-(\text{CH}_2)_8-\text{CH}_2-\text{O}-\text{CH}_2-\text{CH}(\text{OH})-\text{O}-\text{CH}_2-\text{CH}(\text{OH})-\text{CH}_2-\text{SO}_3\text{Na}$
- (8)  $\text{CH}_3-(\text{CH}_2)_8-\text{CH}_2-\text{O}-\text{CH}_2-\text{O}-\text{CH}_2-\text{O}-\text{CH}_2-\text{SO}_3\text{K}$   
1-(dodecyloxydiethyl) oxy-2-potassium sulfonate ethane
- (9)  $\text{CH}_3-(\text{CH}_2)_8-\text{CH}_2-\text{O}-\text{CH}_2-(\text{CHOH})-\text{CH}_2-\text{SO}_3\text{Na}$   
1-oxydodecyl-2,3,4,5-tetrahydroxy-6-sodium sulfonate hexane
- (10)  $\text{CH}_3-(\text{CH}_2)_8-\text{CH}_2-\text{O}-\text{CH}_2-\text{CH}_2-\text{SO}_3\text{Na}$   
1-oxyethyl-2-sodium sulfonate ethane
- (11)  $\text{C}_{10}\text{H}_{21}-\text{CH}(\text{OH})-\text{CH}_2-\text{O}-\text{CH}_2-\text{O}-\text{CH}_2-\text{SO}_3\text{Na}$   
1-(2-hydroxydodecyloxyethyl) oxy-2-sodium sulfonate ethane
- (12)  $\text{CH}_3-(\text{CH}_2)_8-\text{CH}_2-\text{O}-\text{CH}_2-\text{CH}(\text{OH})-\text{O}-\text{CH}_2-\text{CH}(\text{OH})-\text{CH}_2-\text{SO}_3\text{Na}$
- (13)  $\text{CH}_3-(\text{CH}_2)_8-\text{CH}_2-\text{O}-\text{CH}_2-(\text{CHOH})-\text{CH}_2-\text{SO}_3\text{K}$   
1-oxydodecyl-2,3,4,5-tetrahydroxy-6-potassium sulfonate hexane
- (14)  $\text{CH}_3-(\text{CH}_2)_8-\text{CH}_2-\text{O}-\text{CH}_2-(\text{CHOH})-\text{CH}_2-\text{SO}_3\text{Na}$   
1-oxydecyl-2,3-dihydroxy-4-sodium sulfonate butane
- (15)  $\text{CH}_3-(\text{CH}_2)_8-\text{CH}_2-\text{O}-(\text{C}_2\text{H}_4-\text{O})_2-\text{CH}_2-\text{SO}_3\text{Na}$   
1-(decyloxytriethyl)-2-sodium sulfonate ethane
- (16)  $\text{CH}_3-(\text{CH}_2)_8-\text{CH}_2-\text{O}-\text{CH}_2-\text{CH}(\text{OH})-\text{CH}_2-\text{SO}_3\text{Na}$   
1-oxydodecyl-2,3-disodium sulfonate propane

Some of the addition agents of the present invention may be represented by the general formula



wherein R is an alkyl (including hydroxy-alkyl) radical containing at least 6 carbon atoms, in the usual case from 6 to 18 carbon atoms, X is the residue of an aliphatic polyhydroxy substance, Y is a cation, the sulphur of the group  $\text{SO}_3\text{Y}$  being linked directly to carbon of X, and t and w are each integers, preferably 1.

Various of the addition agents of the present invention may also be represented by the general formula



wherein R is an aliphatic radical including or comprising an alkyl (including hydroxy-alkyl) radical having at least 6 carbon atoms, in the usual case from 6 to 18 carbon atoms, n is an integer such as 1, 2, 3, 4 or more, and Y is a cation such as those mentioned hereinabove.

As I have indicated hereinabove and illustrated by some of the examples, various of the addition agents which I have disclosed may be considered as derivatives of aliphatic polyhydroxy substances wherein one or more hydroxy groups are replaced by sulphonic radicals and wherein the hydrogen of at least one hydroxy group of the aliphatic polyhydroxy substances is replaced by an alkyl or hydroxy-alkyl radical containing at least 6 carbon atoms and preferably from 12 to 14 carbon atoms. Among the water-soluble aliphatic polyhydroxy substances, the aforementioned specific derivatives of which are included among the addition agents of my present invention, are, for example, glycerin; glycols such as ethylene glycol, propylene glycol, trimethylene glycol, and the like; polyglycols such as diethylene glycol, triethylene glycol, and the like; polyglycerols such as diglycerol, triglycerol, tetra-

glycerol and mixtures thereof; carbohydrates and sugars such as dextrose, sucrose, and maltose; and sugar alcohols such as arabitol, mannitol, sorbitol, dulcitol, mannitan and sorbitan, and the like.

The alkyl radicals of the addition agents may be selected from a large group including, by way of example, hexyl, heptyl, octyl, nonyl, decyl, undecyl, lauryl, myristyl, cetyl, oleyl, linoleyl, stearyl, ricinoleyl, palmitoleyl; branched chain alkyl such as 2-ethyl hexyl, 2-n-butyl octyl, 2-butyl tetradecyl, and the like.

It will be understood that the addition agents utilized should be soluble in the electrolyte solution at least to such an extent as to fall within the general range as set out hereinabove. In general, the solubility of the addition agents in the electrolyte solutions decreases with the increase of carbon atoms in the alkyl chain of the addition agents and, therefore, lower concentrations of such addition agents may be used. Conversely, higher concentrations, generally speaking, of those addition agents should be used where the number of carbon atoms in the alkyl chain is around 8 to 10 carbon atoms. The addition agents which are preferably employed, as indicated hereinabove, are those having an alkyl chain containing from 10 to 16 carbon atoms and of particular utility are those having an alkyl chain containing predominantly 12 to 14 carbon atoms, the lauryl ether derivatives being especially useful.

Table I sets forth various examples of plating baths with which the addition agents of the present invention may be used effectively to prevent or inhibit pitting. It will be understood that these examples are merely illustrative and are not to be taken as limitative of my invention, it being understood that, in general, the novel teachings of my invention may be utilized in connection with plating baths wherein the addition agents are soluble in the electrolyte solutions to the extent necessary to accomplish the desired results, and wherein said addition agents are not hydrolyzed or otherwise decomposed or modified to an extent sufficient to interfere with their functioning. In general, the addition agents are particularly effective in aqueous acidic electroplating baths wherein the pH of the bath is of the order of about 2 to about 6.

Table I  
In each bath 0.1-0.5 gram/liter or 0.01-0.07 oz./gal. of the compound of Example 1.

|    | Nickel (white)                               | Conc. oz./gal. | Nickel (white)                             | Conc. oz./gal. |
|----|----------------------------------------------|----------------|--------------------------------------------|----------------|
| 60 | $\text{NiSO}_4 \cdot 6\text{H}_2\text{O}$    | 30-40          | $\text{NiCl}_2 \cdot 6\text{H}_2\text{O}$  | 30-40          |
|    | $\text{NiCl}_2 \cdot 6\text{H}_2\text{O}$    | 8              | $\text{H}_3\text{BO}_3$                    | 5              |
|    | $\text{H}_3\text{BO}_3$                      | 5              | Temp. 70-150° F                            |                |
|    | Temp. 100-150° F                             |                | pH=4.0-5.5                                 |                |
|    | pH=4.0-5.5                                   |                | Cathode C. D. 5-150 amp./ft. <sup>2</sup>  |                |
| 65 | Cathode C. D. 5-75                           |                | Cathode C. D. 5-150 amp./ft. <sup>2</sup>  |                |
|    |                                              |                |                                            |                |
|    |                                              |                |                                            |                |
|    |                                              |                |                                            |                |
|    |                                              |                |                                            |                |
|    | Nickel (bright)                              | Conc. oz./gal. | Cobalt                                     | Conc. oz./gal. |
| 70 | $\text{NiSO}_4 \cdot 6\text{H}_2\text{O}$    | 30-40          | $\text{CoSO}_4 \cdot 7\text{H}_2\text{O}$  | 30-40          |
|    | $\text{NiCl}_2 \cdot 6\text{H}_2\text{O}$    | 8              | $\text{CoCl}_2 \cdot 6\text{H}_2\text{O}$  | 8              |
|    | $\text{H}_3\text{BO}_3$                      | 5              | $\text{H}_3\text{BO}_3$                    | 5              |
|    | $\text{C}_6\text{H}_5\text{SO}_3\text{NH}_2$ | 0.3            | $(\text{NH}_4)_2\text{SO}_4$               | 0.2            |
|    | $\text{ZnSO}_4 \cdot 7\text{H}_2\text{O}$    | 0.1            | Temp. 70-120° F                            |                |
| 75 | Temp. 100-150° F                             |                | pH=3.5-5.5                                 |                |
|    | pH=3.5-5.5                                   |                | Cathode C. D. 20-200 amp./ft. <sup>2</sup> |                |
|    | Cathode C. D. 15-75                          |                |                                            |                |

| Nickel-cobalt<br>(bright)                   | Conc.,<br>oz./gal. | Zinc                                        | Conc.,<br>oz./gal. |
|---------------------------------------------|--------------------|---------------------------------------------|--------------------|
| $\text{NiSO}_4 \cdot 6\text{-7H}_2\text{O}$ | 32                 | $\text{ZnSO}_4 \cdot 7\text{H}_2\text{O}$   | 30-40              |
| $\text{CoSO}_4 \cdot 7\text{H}_2\text{O}$   | 8                  | $\text{Zn}(\text{C}_2\text{H}_5\text{O})_2$ | 4                  |
| $\text{NiCl}_2 \cdot 6\text{H}_2\text{O}$   | 6                  | $\text{Al}(\text{SO}_4)_2$                  | 2                  |
| $\text{H}_3\text{BO}_3$                     | 5                  |                                             |                    |
| $\text{HCHO}$                               | 0.15               | Temp. 100-150° F.                           |                    |
| Temp. 100-150° F.                           |                    | pH=4.0-5.5                                  |                    |
| pH=4.0-5.5                                  |                    | Cathode C. D. 10-60                         |                    |
| Cathode C. D. 5-100                         |                    | amp./ft. <sup>2</sup>                       |                    |

| Iron                                      | Conc.,<br>oz./gal. | Copper                                      | Conc.,<br>oz./gal. |
|-------------------------------------------|--------------------|---------------------------------------------|--------------------|
| $\text{FeCl}_2$                           | 40                 | $\text{CuSO}_4 \cdot 5\text{H}_2\text{O}$   | 30-40              |
| $\text{CaCl}_2 \cdot 6\text{H}_2\text{O}$ | 20                 | $\text{Cu}(\text{C}_2\text{H}_5\text{O})_2$ | 4                  |
| Temp. 100-150° F.                         |                    | Temp. 70-150° F.                            |                    |
| pH=3.5-5.0                                |                    | pH=3.0-5.0                                  |                    |
| Cathode C. D. 10-100                      |                    | Cathode C. D. 10-50                         |                    |
| amp./ft. <sup>2</sup>                     |                    | amp./ft. <sup>2</sup>                       |                    |

| Nickel (white)                              | Conc.,<br>oz./gal. | Copper                                    | Conc.,<br>oz./gal. |
|---------------------------------------------|--------------------|-------------------------------------------|--------------------|
| $\text{NiSO}_4 \cdot 6\text{-7H}_2\text{O}$ | 40                 | $\text{CuSO}_4 \cdot 5\text{H}_2\text{O}$ | 30                 |
| $\text{NiCl}_2 \cdot 6\text{H}_2\text{O}$   | 6                  | $\text{H}_2\text{SO}_4$                   | 5                  |
| $\text{H}_3\text{BO}_3$                     | 4-6                | Temp. 80-160° F.                          |                    |
| Temp. 100-180° F.                           |                    | pH=1.0-1.5                                |                    |
| pH=1.5-2.5                                  |                    | Cathode C. D. 20-100                      |                    |
| Cathode C. D. 20-100                        |                    | amp./ft. <sup>2</sup>                     |                    |

While, in the examples listed hereinabove in Table I, I have disclosed the use of the compound of Example 1 as the addition agent, it will be understood that others of the addition agents which I have disclosed may be substituted therefore without in any manner departing from the spirit and teachings of my invention.

It will be understood that, from time to time, more addition agent should be added to replenish that which is lost by "drag-out" or which may possibly be changed, in some manner or other, during the electrodeposition process.

What I claim as new and desire to protect by Letters Patent of the United States is:

1. In a process of electrodepositing metals, the step which comprises electrolyzing an aqueous acid solution of a salt of the metal to be deposited and a minor proportion of a soluble aliphatic alkyl ether sulfonate containing an alkyl radical having a chain of from 6 to 18 carbon atoms, the metal to be deposited being selected from the group consisting of nickel, cobalt, iron, zinc, cadmium, copper, and antimony.

2. In a process for electrodepositing metals, the step which comprises electrolyzing an aqueous acid solution of a salt of the metal to be deposited and a minor proportion of a soluble aliphatic alkyl ether sulfonate containing a straight chain alkyl radical of 12 carbon atoms, the metal to be deposited being selected from the group consisting of nickel, cobalt, iron, zinc, cadmium, copper, and antimony.

3. In a process for electrodepositing metals, the step which comprises electrolyzing an aqueous acid solution of a salt of the metal to be deposited and a minor proportion of a soluble aliphatic alkyl ether sulfonate corresponding to the formula



wherein R is an aliphatic radical comprising an alkyl group of from 6 to 18 carbon atoms, n is an integer, and Y is a cation, the metal to be deposited being selected from the group consist-

ing of nickel, cobalt, iron, zinc, cadmium, copper, and antimony.

4. In a process of electrodepositing nickel, the step which comprises electrolyzing an aqueous acid nickel solution containing a material selected from the group consisting of nickel sulphate, nickel chloride, and mixtures thereof, said aqueous solution also containing a minor proportion of a soluble aliphatic alkyl ether sulfonate containing at least 8 carbon atoms.

5. In a process of electrodepositing nickel, the step which comprises electrolyzing an aqueous acid nickel solution containing a material selected from the group consisting of nickel sulphate, nickel chloride, and mixtures thereof, said aqueous solution also containing a minor proportion of the compound



20 where Y is an alkali metal cation.

6. In a process of electrodepositing metals, the step which comprises electrolyzing an aqueous acid solution of a salt of the metal to be deposited, said solution containing from about 0.1 to about 0.5 gram per liter of a soluble aliphatic alkyl ether sulfonate containing an alkyl group with from 6 to 18 carbon atoms, the metal to be deposited being selected from the group consisting of nickel, cobalt, iron, zinc, cadmium, copper, and antimony.

7. A bath for the electrodeposition of metals comprising an aqueous acid solution of a compound of a metal to be deposited by electrolysis and a minor proportion of a soluble aliphatic alkyl ether sulfonate having an alkyl chain of from 12 to 14 carbon atoms, the metal to be deposited being selected from the group consisting of nickel, cobalt, iron, zinc, cadmium, copper, and antimony.

8. A bath for the electrodeposition of metals comprising an aqueous acid solution of a compound of a metal to be deposited by electrolysis and from about 0.1 to about 0.5 gram per liter of an aliphatic alkyl ether sulfonate containing a straight chain alkyl radical of from 12 to 14 carbon atoms, the metal to be deposited being selected from the group consisting of nickel, cobalt, iron, zinc, cadmium, copper, and antimony.

9. A bath for the electrodeposition of nickel comprising an aqueous acid solution of a material selected from the group consisting of nickel sulphate, nickel chloride, and mixtures thereof, and a minor proportion of a soluble aliphatic alkyl ether sulfonate the alkyl radical of which contains from 8 to 18 carbon atoms.

10. A bath for the electrodeposition of nickel comprising an aqueous acid solution of a material selected from the group consisting of nickel sulphate, nickel chloride, and mixtures thereof, and a minor proportion of the compound



wherein Y is an alkali metal cation.

11. In a process of electrodepositing nickel to obtain a bright or lustrous deposit, the step which comprises electrolyzing an aqueous acid nickel solution containing a metal salt selected from the group consisting of nickel sulphate, nickel chloride, and mixtures thereof, said aqueous solution also containing minor proportions of a soluble aliphatic alkyl ether sulfonate containing an alkyl group having from 6 to 18 carbon atoms.

12. In a process of electrodepositing nickel to obtain a bright or lustrous deposit, the step which

comprises electrolyzing an aqueous acid nickel solution containing a metal salt selected from the group consisting of nickel sulphate, nickel chloride, and mixtures thereof, said aqueous solution also containing minor proportions of an aliphatic alkyl ether sulfonate having at least 8 carbon atoms and a brightener in the form of a compound soluble in the solution and containing the group  $-\text{SO}_2\text{N}-$ .

13. A bath for the electrodeposition of nickel in the form of a bright or lustrous deposit, comprising an aqueous acid solution of a material selected from the group consisting of nickel sulphate, nickel chloride, and mixtures thereof, and minor proportions of a soluble aliphatic lauryl ether sulfonate.

14. A bath for the electrodeposition of nickel in the form of a bright or lustrous deposit, comprising an aqueous acid solution of a material selected from the group consisting of nickel sulphate, nickel chloride, and mixtures thereof, and minor proportions of a soluble aliphatic lauryl ether sulfonate and a brightener in the form of an aromatic compound soluble in the solution and containing the group  $-\text{SO}_2\text{N}-$ .

15. In the process of electrodepositing metals, the step which comprises electrolyzing an aqueous acid solution of a salt of the metal to be deposited and a minor proportion of a soluble

aliphatic alkyl ether sulfonate corresponding to the formula:



5 wherein R is an alkyl radical containing from 6 to 18 carbon atoms, X is the residue of an aliphatic polyhydroxy substance, Y is a cation, the sulphur of the group  $\text{SO}_3\text{Y}$  being linked directly to carbon of X, and t and w are each integers, the metal to be deposited being selected from the group consisting of nickel, cobalt, iron, zinc, cadmium, copper, and antimony.

16. A bath for the electrodepositing of metals comprising an aqueous acid solution of a compound of the metal to be deposited by electrolysis and a minor proportion of a soluble aliphatic alkyl ether sulfonate corresponding to the formula:



20 wherein R is an alkyl radical containing from 6 to 18 carbon atoms, X is the residue of an aliphatic polyhydroxy substance, Y is a cation, the sulphur of the group  $\text{SO}_3\text{Y}$  being linked directly to carbon of X, and t and w are each integers, the metal to be deposited being selected from the group consisting of nickel, cobalt, iron, zinc, cadmium, copper, and antimony.

HENRY BROWN.